

## UNITED STATES PATENT OFFICE

2,321,347

## PHOTOGRAPHIC FIXING BATH

James R. Alburger, Merion, Pa., assignor to Radio Corporation of America, a corporation of Delaware

No Drawing. Application November 30, 1939,  
Serial No. 306,971

4 Claims.

(Cl. 95—88)

This invention relates to an improved photographic fixing bath, and more particularly to a fixing bath which is adapted for use at abnormally high temperatures and which can be used after the use of a highly alkaline developer without causing reticulation.

The usual types of fixing baths are either practically neutral or are somewhat acid and include, in addition to the sodium thiosulphate, which dissolves the undeveloped silver salts, an acid sodium salt or similar acidifying agent and a hardening agent. If a film has been dissolved in a highly alkaline developer or has been developed at an unusually high temperature so that the gelatine is considerably softened and it is then placed in such a fixing bath, the sudden hardening of the surface accompanied by the acidifying thereof which causes a sudden contraction of the surface layer of the gelatine in relation to the lower layers has a tendency to cause reticulation. I find, however, that if the developed film is placed in a fixing bath having an alkalinity approaching that of the developer no such reticulation occurs and a correspondingly improved photographic image results.

If an appropriate alkali is added to a sodium thiosulphate solution of ordinary concentration, it tends to soften the emulsion and render the film liable to damage in handling, and reticulation is likely to occur when the film is placed in the succeeding wash. The addition of an ordinary hardening agent to such a fixing bath does not prevent this difficulty, since the softening of the gelatine occurs before the hardening agent has time to become effective.

I secure the necessary degree of alkalinity without the foregoing objections and with a hardening, instead of a softening of the gelatine by balancing the alkali with alum. The alum reacts with the alkali to first form aluminum hydroxide, which tends to be precipitated and to then form an aluminate which remains in solution, but which has a hardening action on the gelatine. If the alkali is used up by oxidation, or otherwise, a corresponding amount of aluminum hydroxide is precipitated, thereby maintaining the alkalinity of the bath constant.

One object of the invention is to provide an improved fixing bath.

Another object of the invention is to provide a fixing bath which may be used at relatively high temperatures.

Another object of the invention is to provide a fixing bath which will prevent reticulation of

the emulsion when either the developer or fixing bath are used at high temperatures.

Another object of the invention is to provide a fixing bath which will automatically recover the dissolved silver.

Other and incidental objects of the invention will be apparent to those skilled in the art from a reading of the following specification.

In the preparation of my improved fixing bath 10 I use the usual sodium thiosulphate as a fixer, and I may also add paraformaldehyde as an additional hardener. The balancing of the alkali and alum may be accomplished as described and claimed in my applications Serial No. 15 205,362 and 205,363, both filed April 30, 1938, now U. S. Patents Nos. 2,199,903 and 2,199,904, respectively, of May 7, 1940, which describe such a balanced solution of alkali and alum applied to a developer.

20 A typical formula for my improved fixing bath is as follows:

|                     |          |
|---------------------|----------|
| Sodium thiosulphate | 400      |
| Alum                | 40-26    |
| Sodium hydroxide    | 30-20    |
| Para-formaldehyde   | grams 20 |
| Water               | cc 1000  |

The proportion of alum and sodium hydroxide is, as indicated above, in the general ratio of 4:3. The quantity of sodium hydroxide used, however, is determined by the alkalinity of the developer which preceded the fixing bath. If the developer is highly alkaline, the fixing bath should have substantially the same alkalinity which can be determined as usual by the pH value. Since there is no change in the alkalinity of the solution in which the film is immersed, there is then no tendency toward reticulation in passing the film from one solution to the other, while the hardening action of the fixing bath is sufficient to prevent any tendency toward reticulation when the film is immersed in the subsequent wash water.

As pointed out above, there is a tendency for the alkali in the fixing bath to be gradually oxidized by the air in contact with the surface thereof, and particularly when used for developing motion picture film, by the air carried into the bath by the film, and this oxidation releases a corresponding amount of aluminum hydroxide from solution. This aluminum hydroxide settles out in the form of a gelatinous precipitate. Since the fixing bath is alkaline and not acid, it does not suddenly stop the action of new developer 55 in the emulsion, as would an acid fixing bath.

The consequence of this is that any developer in the emulsion goes into solution in the fixing bath and reduces the dissolved silver in the fixing bath. This reduced silver, which is practically in colloidal form, is precipitated with the aluminum hydroxide and the silver may be readily recovered from the resulting sludge. A further result of this action is that the fixing bath does not become saturated with silver salts and maintains its original activity over a relatively long time. If an insufficient quantity of developer to accomplish the regeneration of the fixing bath is carried over by the film, small additional quantities of developer may be added to the fixing bath for this purpose, and partly spent developer may be used, thereby recovering not only the silver in solution in the fixing bath, but also that in solution in the developer.

It will be apparent to those skilled in the art that the proportion of sodium thiosulphate or "hypo" in the solution may be varied according to the requirements of the work at hand, and it will be also apparent that not only should the alkalinity be varied as pointed out, but that the quantity of para-formaldehyde should be varied according to the degree of hardening desired. Ordinary formaldehyde may, of course, be added

5 to the bath instead of the para-formaldehyde, but there is no point to such procedure since the formaldehyde is converted into the para-formaldehyde, and this procedure has the disadvantage that the hardening action varies according to the degree to which the polymerization has occurred.

I claim as my invention:

10 1. A photographic fixing bath containing a solvent of silver salts, an alum, and sufficient alkali to dissolve the aluminum compound tending to be precipitated by the alkali.

15 2. A photographic fixing bath containing a solvent of silver salts, an alum, sufficient alkali to dissolve the aluminum compound tending to be precipitated by the alkali, and a hardening agent.

3. A photographic fixing bath containing sodium thiosulphate, an alum, and sufficient alkali to dissolve the aluminum compound tending to be precipitated by the alkali.

20 4. A photographic fixing bath containing sodium thiosulphate, a solvent of silver salts, an alum, sufficient alkali to dissolve the aluminum compound tending to be precipitated by the alkali and a hardening agent.

25 JAMES R. ALBURGER.